

J. S. KRUSE.

FORMATION OF BLOCKS OR THE LIKE SUITABLE FOR ROAD OR OTHER PURPOSES.

APPLICATION FILED MAR. 28, 1912.

1,082,752.

Patented Dec. 30, 1913.



Fig. 1.



Fig. 2.

Attest:

John S. Kruse,  
C. E. Parsons

Inventor:

Johann S. Kruse,  
by John Middleton Donaldson, his  
Attest.

# UNITED STATES PATENT OFFICE.

JOHANN SECUNDUS KRUSE, OF KENSINGTON, LONDON, ENGLAND.

## FORMATION OF BLOCKS OR THE LIKE SUITABLE FOR ROAD OR OTHER PURPOSES.

1,082,752.

Specification of Letters Patent. Patented Dec. 30, 1913.

Application filed March 28, 1912. Serial No. 686,725.

To all whom it may concern:

Be it known that I, JOHANN SECUNDUS KRUSE, a subject of the King of Great Britain and Ireland, and residing at 48 Elm 5 Park Gardens, Kensington, in the county of London, England, have invented a certain new and useful Improvement in and Relating to the Formation of Blocks or the like Suitable for Road or other Purposes, of 10 which the following is a specification.

This invention relates to blocks or the like particularly suitable for use as road blocks, and has for its object to provide an improved road block containing bituminous 15 matter which shall be comparatively cheap to manufacture and effective and lasting in wear.

The invention consists in a block or the like for use on roads or for other purposes, 20 for instance crushed as a substitute for macadam, and herein referred to as a "road block" of the kind formed from a bituminous body, a body containing sulfur and any desired filling, heated to a suitable temperature 25 of for example 250° F. which is subjected to a pressure of about four tons per square inch or over.

The invention also consists in a road block formed of the following bodies in substantially 30 the proportions given namely clinker 78½%; Lake Trinidad asphaltum 19½%; sulfur 1½% and mineral oil ½% subjected to a suitable temperature for melting the asphaltum and sulfur, the composition being thoroughly 35 mixed and subjected to high pressure, namely about five tons per square inch.

The invention also consists in the road block compositions herein described.

Referring to the accompanying diagrams, 40 Figure 1 is a curve formed of the average of some experiments showing the relation between the tons per square inch to which the block is subjected during manufacture and the tons per square inch which it will stand on crushing. Fig. 2 contains the 45 results of experiments to test the wear of blocks included in the present invention and shows the relation between the tons per square inch pressure to which they were subjected in making and the percentage loss after a four hour test.

As the result of a large number of experiments which I have carried out I find that the best block, that is to say the one 55 which has the highest resistance to crushing consistent with good wear and with rea-

sonable cost of production is formed of clinker, Lake Trinidad asphaltum, flowers of sulfur and heavy mineral oil. Convenient quantities for a small test block are:— 60

|                         |     |       |   |         |
|-------------------------|-----|-------|---|---------|
| Clinker                 | 256 | grams | = | 78.2%   |
| Lake Trinidad asphaltum | 64  | "     | = | 19.6%   |
| Sulfur                  | 5   | "     | = | 1.5%    |
| Mineral oil             | 2   | "     | = | 0.6% 65 |

The clinker I have employed is crushed and sifted through a sieve having twenty-two meshes to the inch. I find it convenient to raise the temperature of the clinker, asphaltum and oil to such value as to enable proper mixing to be obtained; for instance up to 380° F. after which the sulfur can be stirred into the incorporated mass and then mixed therewith for about a minute. The 70 mixture is next removed to a press carefully heated and then subjected to a high pressure, for instance 4 to 5 tons per square inch, after which it can immediately be taken from the press and the block thus 75 formed allowed to cool.

In Fig. 1 the average result of certain experiments is shown. The blocks used in these experiments were compounded according to the formula just given and after they 80 had stood for a day or so they were subjected to a crushing test. It will be seen that increasing the pressures used in the manufacture of the blocks up till about 4 tons per square inch enables blocks of correspondingly increased strength to be obtained. After this with a pressure say up till about 85 6 tons per square inch a slight increase is found but this is not so marked whereas after this figure increase of pressure during 90 making produces substantially no gain of strength. It will thus be understood that the use of high pressures of the order of 95 4-6 tons per square inch during manufacture is useful and efficient particularly compared with blocks produced under lower pressure or no pressure at all. Further, although the pressure may be increased above this value there is no corresponding gain in efficiency. I also find as the result 100 of experiments that the resistance of a block to crushing is very akin to its resistance to wear and tear. I have subjected a number 105 of blocks to a test comprising the frictional contact of the blocks with flint stones in a rotating rumble and have found that after a run of some hours the percentage loss in

weight of the blocks formed under low pressures is very much greater than those formed under high pressures, the change being very marked up till about 4 tons per square inch 5 as in the crushing test, but being very much smaller after this point had been reached. The result of an experiment on a four hour test is shown in Fig. 2 and it will be seen that the bend of the curve occurs in substantially the same place as the bend of the curve in Fig. 1.

It will be understood that the manner of carrying the invention into effect and the compositions referred to above are given 15 by way of example only and may be modified as desired; for instance either pure bitumen or bituminous rock may be used the formulas being modified to take account as regards bitumen only of the part of the 20 rock which contains bituminous matter, the remainder being counted as filling. Further, although a small quantity of oil such as a heavy mineral oil may be included it may be omitted if desired. It is more particularly useful with bituminous rocks because there is usually oil of some kind present in bitumen that has been refined. I find the quantity of oil added should not generally exceed 3% by weight of the whole 25 block, the actual amount depending on the nature of the bitumen, that is whether it is fluid, soft or the reverse.

As regards the proportions of materials referred to in the above examples these may 30 be varied but I find that broadly speaking the proportion of sulfur or the corresponding amount of other vulcanizing agent should not be greater than 20% of the bitumen and not less than about 5%. With 35 values less than this the block ordinarily is too soft and with higher values becomes too brittle, although when the amount of bituminous matter and sulfur is small with regard to the amount of filling for instance 40 in blocks of the kind referred to with reference to Figs. 1 and 2 I find that the sulfur may be used in quantity between about 10-20% of the amount of the bitumen without seriously affecting the crushing strength 45 of the completed block either to its improvement or detriment. As to the proportion of bituminous matter which can be used I prefer to employ about 20-25% of the total mass but more or less may be used.

50 I find that with the formula containing clinker and asphaltum reducing the amount of asphaltum to 46 grams causes the resistance to crushing to be reduced 50 to 60% while increasing the quantity to 80-90 grams 55 does not give a proportionate increase in strength.

It will be understood that a flint filling or other fillings may be employed such as sand, slag, clinker, slate, stone or the like, for example and it is generally preferable to use 60

the filling in a form containing particles of about the size of sand grains although larger particles may be used if desired. If desired mixing can be effected in a jacketed mixer and the material can all be mixed together or the bitumen can be melted and then the sulfur stirred in afterward. Further the heating may be conducted in open or closed vessels and may be carried on for any suitable time, and it is preferable during the 75 whole time to keep the temperature comparatively high for instance between the limits 270° F. to 360° F.

70 As indicated above I prefer to subject the mixture to a pressure reasonably high say 4 or 5 tons to the square inch although if desired I may utilize considerably higher pressures and may adjust the amount of bitumen for example according to the pressures employed, the kind or quality of block desired 80 or the time during which the pressure is exerted. In place of part or the whole of the bitumen a vegetable pitch may be employed such as plastic pitch.

Having now described my invention what 85 I claim as new and desire to secure by Letters Patent is:—

1. A process for the production of road blocks and the like which consists in incorporating with heat a bituminous body, a 90 body containing sulfur and a suitable filling material and subsequently subjecting the mixture to a pressure of about four tons per square inch; as set forth.

2. A process for the manufacture of road 100 blocks and the like consisting in incorporating together with heat the following materials in substantially the proportions specified, viz:—clinker 78½%, asphaltum 19½%, sulfur 1½%, mineral oil ½%, and subsequently subjecting the mixture to a pressure of at least four tons per square inch; as set forth.

3. A process for the manufacture of road 110 blocks and the like which consists in mixing a bituminous matter and a filling material under the action of heat, adding a sulfur body thereto and incorporating same therewith and subsequently subjecting the mixture to pressure of at least about four tons 115 per square inch; as set forth.

4. A process for the manufacture of road 120 blocks and the like which consists in heating a bituminous body and a filling material to about 400° F. and effecting mixture thereof, adding a sulfur body and incorporating the same with the mass, after which the mixture is subjected to pressure of about four tons per square inch; as set forth.

5. A road block and the like formed by a 125 bituminous body, a vulcanizing body and a filling material in substantially the following proportions, viz:—bituminous matter 20-25%, vulcanizing material 1-5%, filling 79-70%, which is highly compressed; said 130

block being capable of resisting a crushing stress of about two tons to the square inch, substantially as described.

6. A road block and the like formed from a bituminous body, a body containing sulfur and a suitable filling material which is highly compressed, the proportion of sulfur being between 5 and 20% of bitumen; said block losing less than about 10% by

weight in a four hour wearing test, substantially as described.

In testimony whereof, I affix my signature in presence of two witnesses.

JOHANN SECUNDUS KRUSE.

Witnesses:

PERCY RAYNER SMITH,  
P. R. OUTHWARTE.